

Nov. 25, 1941.

T. H. SWAN

2,264,224

MULTIPLY LAUNDERABLE APPAREL AND PROCESS OF PREPARING SAME

Filed Feb. 5, 1935

Fig. 1



Fig. 3



Fig. 2



Fig. 4



Fig. 5



Inventor

Thomas H. Swan

By

E. C. Danborn

Attorney

## UNITED STATES PATENT OFFICE

2,264,224

MULTIPLY LAUNDERABLE APPAREL AND  
PROCESS OF PREPARING SAMEThomas H. Swan, Pittsburgh, Pa., assignor to  
Cluett, Peabody & Co., Inc., Troy, N. Y., a cor-  
poration of New York

Application February 5, 1935, Serial No. 5,105

15 Claims. (Cl. 154—2)

This invention relates to wearing apparel of the type adapted to be laundered, and more particularly to wearing apparel such as shirts, collars, cuffs, plaits and the like, as forming part of such wearing apparel.

There are several types of fabric garments manufactured according to the present state of the art as, for example, those which are manufactured and worn in the untreated state, that is, the collars and cuffs have no stiffening agent; those having collars and cuffs and similar exposed portions stiffened with a temporary stiffening agent such as starch; those having collar and cuff units stiffened by partial parchmentization, by means of suitable reagents, and those in which starched interlinings are used as stiffeners. Further, cellulose derivative coated fabrics have been proposed as stiffening interlinings in collars and cuffs; garments in which the component fabrics of the collars and cuffs are laminated by means of cellulose derivative compositions have also been made.

Of these various types mentioned, none are entirely satisfactory; those garments which are made of untreated fabrics soil quickly and wrinkle easily. The starched type, while presenting a very satisfactory initial appearance, is sensitive to spotting by water and soon becomes wilted and wrinkled especially in warm weather. The collars and cuffs of two-ply and multi-ply construction, the fabrics of which are laminated and stiffened by partially parchmentizing the fabrics with acid, have the disadvantage of lowered tensile strength and unsatisfactory wearing qualities. In the case of the wearing apparel having the interlinings pre-stiffened with starch, for example, the treatment is effective only until the first laundering which removes the starch. While the collars or cuffs can, of course, be restiffened by treatment with starch, they do not retain their appearance for any length of time, particularly in summer weather. Where certain cellulose derivative coated fabric interlinings are used the result is not satisfactory because of the tendency for the coating to disintegrate and disappear and often to discolor when the garment is subjected to laundering processes. The same condition prevails with respect to collars and cuffs in which the component fabrics are laminated directly by means of the common cellulose derivative compositions.

This invention has as an object the provision of wearing apparel having collars, cuffs and the like which are non-wrinkling, readily cleanable by washing or dry cleaning and capable of re-

taining their shape after laundering without being subjected to a subsequent stiffening operation.

5 A further object is the provision of a multiply collar or cuff and the like which upon repeated launderings and pressings, will not show the characteristic "stitch pucker" of present day wearing apparel.

A still further object is the production of collars 10 which will resist distorting influences and will tend to resume their original appearance when the distorting force is removed.

These objects are accomplished in the present invention by uniting specially treated fabrics in 15 laminated relation and more particularly by first coating one or more fabrics with an adhesive composition, preferably drying to expel the volatile materials present in the adhesive in cases where the adhesive contains volatile material, 20 placing the fabrics in contact with each other to subject the contiguous surfaces thereof to the action of the adhesive, and joining by means of heat and pressure.

The general construction of the wearing apparel described in the present invention will be 25 readily apparent by reference to the drawing.

In the drawing Figure 1 is a diagrammatic sketch of a three-ply collar laid flat. Figure 2 represents a cross section through the collar 30 along the line 2—2 in Figure 1, on an enlarged scale. Figure 3 indicates, on an enlarged scale, the assembly of the parts before forming the collar. Figure 4 is a sketch of a shirt showing 35 a collar, plaits and cuffs embodying the present invention. Figure 5 represents a dress shirt in which the bosom has been made semi-stiff by the invention disclosed herein. In all the figures the outer or facing fabrics are indicated as 1. The adhesive is shown at 2 while 3 is the innerliner and 4 is stitching.

40 In order that the construction of the wearing apparel of the invention may be more fully understood, the following definition of terms used is given.

45 By a three-ply collar is understood a construction in which an extra layer of fabric, usually of a cheaper and coarser grade, is interposed between the fabrics in a "fold over" collar, the function of this intermediate layer being to add 50 stiffness, thickness, and general body to the article. This ply is indicated as interlining 3 of the drawing.

55 By the term "semi-stiff" or "stiffened" as applied to an article of apparel is understood one having a pliability or "hand" intermediate an

unstarched, untreated article on the one hand, and a fully starched article on the other hand.

The practice of the present invention may be illustrated in the preparation of a three-ply collar, in which an interlining, which is usually a cotton fabric of cheap construction, is coated with a thermoplastic adhesive composition. This composition may be one of those referred to hereinafter. The interlining, for example, may be a sheeting weighing 4.7 oz. per yard and having a thread count of 49 warp threads and 54 filling threads. This is coated on both faces with adhesive in any convenient way, as, for example, by means of a doctor knife, squeeze rollers, spraying equipment, or by any of the methods known to those skilled in the art of coating fabrics. The adhesive is then preferably allowed to dry, which may be accomplished either in the air at room temperature or by heating in an oven. The collar may then be assembled by placing the two outer fabrics, which may be broadcloth, madras or the like, on top of the coated interlining and assembling the parts by stitching. The collar is then turned inside out in such a way that the interlining will fall between the two layers or plies of broadcloth, madras or the like. The joining of the parts is then carried out by applying heat and pressure simultaneously; as, for example, by ironing at normal ironing temperatures and pressures, or by applying higher temperatures and/or pressures in any suitable way, it being sufficient simply that the temperatures and pressures employed be adequate to render the interlining coating sufficiently plastic and adhesive to cause the fabric plies to be united. The collar may be decorated by ornamental stitching along the edges, if desired, which stitching may be done either before or after the plies are cemented. The edge of the collar which is to be attached to the neck-band may be either stitched ornamenteally or such stitching may be omitted therefrom. The collar is affixed to the neck-band in the usual manner. The neck-band may be either of conventional construction or may be formed by uniting fabric plies in laminated relation through a thermoplastic adhesive in the same manner as above described with respect to the collar proper.

Wearing apparel having more or less than three plies may be prepared in a similar manner, as will be evident to those skilled in the art. It is apparent, for example, that where two plies are to be united, one or both may be coated with adhesive, the latter then preferably dried, and the plies then placed appropriately in contact, with the adhesive therebetween, after which they may be firmly united by the simultaneous application of heat and pressure. In an alternative mode of assembly of two component pieces of adhesive coated fabric to form a collar, for example, the adhesive coated pieces or plies may be placed with their uncoated surfaces in contact, then stitched together, and then turned inside out so as to bring the two adhesive coated surfaces together, inside the collar, after which the joining of the parts may be accomplished by applying heat and pressure simultaneously. It will be obvious that my invention is not limited to the joining in laminated relation of any particular number of plies.

The adhesive composition employed may be of any of the known types which are thermoplastic, and especially those which are resistant to normal laundering operations. By "resistant to normal laundering operations," I mean substan-

tially unsusceptible to undesirable changes or objectionable deterioration under the influence of the reagents (such as the detergents and bleaching agents) and other conditions present in laundering processes as commonly practiced. As employed in this specification and the ensuing claims, the term "thermoplastic adhesive" and like expressions refer to a substance which, as its temperature is elevated, has its adhesiveness increased sufficiently to enable it to firmly bond or unite fabrics under the influence of heat and pressure, and which retains its bonding capacity after its temperature is lowered, said substance furthermore remaining thermoplastic at normal ironing temperatures so as to be repeatedly resoftenable at those temperatures to effect re-bonding in the event of separation of the fabrics.

The adhesive which I prefer employing, furthermore, while having its plasticity or flow capacity increased under rise in temperature, is nevertheless sufficiently flow-resistant at the boiling temperature of water that migration of the adhesive through the interstices of the fabric is prevented. It is, however, thermoplastic at normal ironing temperatures, such, for example, as of the order of 250°-350° F. With such an adhesive, if for any reason the bond between the fabric plies of a collar or other article is loosened during laundering, as by rubbing or agitation, such bond is re-established during ironing of the article. The pressures applied to insure joining of the fabric plies by the thermoplastic adhesive may vary from hand pressures applied to the ordinary flat iron to pressures obtained in machine presses, pressures within the range from a few pounds per square inch to several thousand pounds per square inch being suitable. The adhesive should, moreover, preferably retain the characteristic of thermoplasticity adequate for uniting fabric plies under heat and pressure, despite exposure of the adhesive to air, moisture, or to ordinary laundering conditions.

The following composition has been found satisfactory as the thermoplastic adhesive mentioned above. The figures represent percentage by weight.

|                   |      |
|-------------------|------|
| Resoglaz *        | 8.5  |
| Diethyl phthalate | 1.5  |
| Benzene           | 85.0 |
| Xylene            | 5.0  |

\* Polymerized styrene.

Other thermoplastic resins may be used in place of the Resoglaz, for example, vinyl resins, particularly those prepared by the joint polymerization of the vinyl acetate and vinyl chloride. The acetate is usually present in amounts from 20 to 70 percent of the chloride. The proportions of the esters depend upon the properties desired in the adhesive as will be apparent to those skilled in the art. Similarly the amount of plasticizer and solvent can be regulated to suit the desired degree of stiffness wanted in the finished product and the fineness of the weave of the fabrics used.

Other resins which may be employed are thermoplastic resins of the phenol-formaldehyde group, thermoplastic resins included in the polyhydric alcohol-polybasic acid class, or thermoplastic resins in the toluene sulfonamide-formaldehyde group.

The purpose of the volatile solvent in those compositions in which it is used is primarily to act as a carrier for the solid constituents of the

adhesive. The volatile material need not be relied upon to effect the final adhesion of the fabrics and may be substantially entirely removed by drying as previously described. At the same time, it is to be understood that the invention is not restricted to the bonding of fabrics by thermoplastic adhesives from which the solvent has been substantially entirely removed; and instead substantial amounts of solvent, either originally present or added at the time of combining, may, if desired, be present at the time the adhesive is subjected to heat and pressure for uniting the fabrics. The use of volatile solvents in certain instances permits the deposition of a smooth film of the thermoplastic material and also assists in the ease of applying the adhesive to certain types of fabrics. The resin may also be cast in sheet form and inserted between two or more of the plies.

It is understood that various modifications with regard to solvents used will be readily apparent to those skilled in the art. For example, such solvents as ethyl acetate or other esters as butyl propionate, isopropyl acetate; ethyl methyl ketone, etc. may be appropriately used. In general, the choice of volatile solvents will be governed by the degree of solubility of the constituents of the adhesive, the rate of removal of the volatile material desired and also economic factors. Also, various modifications with respect to plasticizers may be made and any of a wide variety of well known plasticizers, such as tricresyl phosphate, for example, may be used.

Inorganic pigments, such as titanium dioxide or barytes, may be used; and further, mineral pigments which are either translucent or opaque, white or colored, may be introduced into the adhesives. The use of barytes is advantageous in certain instances because combinations of the type described yield a translucent film.

No limitation is placed on the type of fabric which may be used in the construction of the wearing apparel which is described in the invention. Common types of cotton fabrics used for producing collars, cuffs, plaits of shirts, and the like, wearing apparel such as broadcloth, madras, oxford cloth, etc., may be used with equal satisfaction. Further, silk fabrics and various types of fabrics woven from synthetic yarns such as are made from regenerated cellulose, cellulose acetate, cellulose nitrate, cuprammonium cellulose, etc., are included within the scope of the invention. Linen fabrics, as well as other natural type yarn fabrics, may also be used.

In the carrying out of the invention it will be apparent that fabric sheets, after being coated and dried, may be rolled up and stored until required for assembly into the desired articles. The plies requisite for the formation of the desired collar or any other article may of course be cut from sheets of the respective fabrics in any convenient way, as by suitable dies, and then placed together and united in the manner described above.

The product of the invention finds wide use as a component part of shirts of the negligee type where it is desirable to have a garment retain its crisp freshly laundered appearance even under conditions of very warm weather and high humidity when the ordinary type of garments are found to wilt, wrinkle and become unsightly from the moisture of the atmosphere and perspiration of the wearer. As previously indicated, in addition to collars and cuffs on shirts and similar wearing apparel, the product of the invention

finds itself applicable to the manufacture of plaits and demibosoms in the shirt industry, and is also particularly adapted for collars, cuffs and other exposed portions of nurses', chauffeurs' and maids' uniforms and the like. The invention finds further application in the manufacture of neckties of various types where several plies of suitable fabric are laminated to yield a non-wrinkling cravat. Because of the unique properties presented by the product of the invention, many other uses will suggest themselves to those skilled in the art.

Garments which have collars, cuffs, demibosoms, plaits and the like made according to the present invention present the advantages of ease of cleanability, and extreme resistance to crumpling and wilting when in contact with moisture. In addition to these properties, collars and the like will retain the starched appearance after the initial assembly of the collar, no special treatment or equipment being required to keep the collar in its intended condition. "Stitch pucker," a fault common in collars of the soft variety, is eliminated in the present invention because the plies are rigidly joined throughout the surface, and even the stitching tends to become thoroughly anchored and embedded in the adhesive.

The products of the invention present as an additional advantage the ability to be laundered and pressed without being restiffened by means of starch or similar stiffening agents. The products may be subjected to repeated launderings and pressings and at the same time present a satisfactory and desirable appearance.

While I have disclosed my invention with respect to collars, cuffs, and the like, I do not wish to confine it to the manufacture of these specific pieces of apparel. For example, I have also found that suits of linen, cotton, light-weight wool or other similar fabrics may have the lapels and collars of the coat and the cuffs of the trousers treated as above described. I may also cement the fabrics making up the lapel and collar of rain-coats, particularly of gabardine material. The advantage in this application consists primarily in that the lapel will not pucker when sewed or when the garment becomes wet from rain. The adhesives disclosed above are not affected by ordinary dry cleaning methods and any garment which is so cleaned and pressed will have a neat and orderly appearance.

The viscosity or flow-resistance of the adhesive employed should be such that when the fabric is subjected to heat and pressure, the adhesive will not strike through and stick to the heating iron and rolls; and hence, when the fabric to be treated is of a very open or porous weave the viscosity of the adhesive should be correspondingly increased. The proper viscosity can easily be determined by trial with the selected fabric and it will be evident to those skilled in the art that the characteristics of the adhesives employed can be varied to meet the requirements of the particular fabrics utilized. However, good results will be obtained if the examples are followed.

The invention also contemplates the application of the thermoplastic adhesives to the fabric plies in spaced dots, lines, or other spaced portions, instead of in a continuous coating. This may be accomplished in any convenient way, as by rollers grooved or having suitably spaced projections.

It is apparent that many widely different em-

bodiments of this invention may be made without departing from the spirit and scope thereof and, therefore, it is not intended to be limited except as indicated in the appended claims.

I claim:

1. Process of preparing semi-stiff portions of wearing apparel of the class described which comprises coating an interliner fabric with a composition comprising a polymerized mixture of vinyl acetate and vinyl chloride, solvent, and plasticizer, allowing the same to dry, applying thereto fabrics on top of said interliner, stitching along the edges of the same, reversing the position of the fabrics so that the interliner will be between the face and back fabric and joining parts by means of heat and pressure.

2. Process of making collars, cuffs and the like, which comprises applying to a suitable fabric a thermoplastic adhesive comprising a resin polymer (approximately 80% vinyl chloride and 20% vinyl acetate), ethyl methyl ketone, tricresyl phosphate, and titanium dioxide, allowing the adhesive to dry, cutting a desired pattern from the fabric, interposing said pattern as an interlining between two fabrics forming the face and back of the finished collar, cuff or the like, stitching said fabrics along their edges and subjecting the assembled fabrics to heat and pressure whereby the adhesive is softened and upon cooling forms a bond between the surfaces of the

3. An article of launderable apparel comprising a plurality of fabric layers joined by means of a non-cellulosic composition wherein the major non-volatile ingredient comprises a thermoplastic synthetic resin having the property of becoming plastic to effect bonding under the sole action of heat and pressure and of remaining thermoplastic to effect rebonding under subsequent applications of heat and pressure alone at normal ironing temperatures, said resin being substantially insoluble in hot water.

4. A semi-stiff collar comprising fabric plies united by an adhesive comprising a thermoplastic synthetic resin substantially insoluble in hot water, said resin also having the property of becoming plastic and effecting bonding under the sole action of heat and pressure and of remaining thermoplastic to effect rebonding under subsequent applications of heat and pressure alone if the bond becomes loosened, said adhesive being sufficiently flow-resistant to avoid striking through the fabric upon the application of heat and pressure to effect bonding of the plies.

5. A semi-stiff collar as defined by claim 4, wherein the resin is a vinyl resin.

6. An article of apparel of the class consisting of collars, cuffs and shirts, said article comprising fabric plies united by means of a thermoplastic vinyl resin capable in and of itself of effecting rebonding by the sole action of heat and pressure at normal ironing temperatures.

7. Process of preparing multi-ply collars, cuffs and the like, which comprises coating a sheet of intermediate ply material with a solution of a thermoplastic synthetic resin substantially insoluble in hot water and having the property of becoming plastic to effect bonding by the sole action of heat and pressure and of remaining thermoplastic to effect rebonding under subsequent application of heat and pressure alone, allowing the solvent to evaporate, cutting out an interliner from said sheet, and firmly bonding thereto a face and back ply by means of heat and pressure.

8. A semi-stiff collar comprising fabric plies united by an adhesive comprising a thermoplastic synthetic resin having the property of becoming plastic and effecting bonding under the sole action of heat and pressure and of remaining thermoplastic to effect rebonding under subsequent applications of heat and pressure alone if the bond becomes loosened, said adhesive being sufficiently flow-resistant to avoid striking

5 through the fabric upon the application of heat and pressure to effect bonding of the plies, said resin being selected from a group consisting of polymerized styrene and a co-polymer of vinyl acetate and vinyl chloride.

10 15 9. An article of apparel of the class consisting of collars, cuffs and shirts, said article comprising fabric plies united by means of a thermoplastic synthetic resin capable in and of itself of effecting rebonding by the sole action of heat and pressure at normal ironing temperatures, said resin being selected from a group consisting of polymerized styrene and a co-polymer of vinyl acetate and vinyl chloride.

20 25 10. An article of apparel of the class consisting of collars, cuffs and shirts, said article comprising fabric plies united by means of a thermoplastic vinyl resin capable in and of itself of effecting rebonding by the sole action of heat and pressure at normal ironing temperatures, said resin being one resulting from the joint polymerization of vinyl acetate and vinyl chloride, with the chloride predominating.

30 35 11. An article of apparel of the class consisting of collars, cuffs and shirts, said article comprising fabric plies united by means of a thermoplastic vinyl resin capable in and of itself of effecting rebonding by the sole action of heat and pressure at normal ironing temperatures, said resin being a co-polymer of vinyl acetate and vinyl chloride.

40 45 12. An article of apparel of the class consisting of collars, cuffs and shirts, said article comprising fabric plies united by an adhesive comprising a thermoplastic synthetic resin which is solid at room temperatures and flexible in thin sheets, said resin being adhesive to said fabric upon becoming softened under the sole action of heat and pressure at normal ironing temperatures and under ironing pressures, and also remaining thermoplastic under repeated heating at ironing temperatures, said resin being also substantially insoluble in hot water and sufficiently flow-resistant at the temperature of boiling water to prevent migration of said substance through the interstices of said fabric.

50 55 60 65 70 75 13. An article of launderable apparel comprising a plurality of fabric layers joined by an adhesive comprising a thermoplastic synthetic resin having the property of becoming plastic to effect bonding under the sole action of heat and pressure at a temperature within the range of about 250°-350° F. and at a pressure within the range of ironing pressures and of remaining thermoplastic to effect rebonding under subsequent applications of heat and pressure alone at a temperature within said temperature range and a pressure within said pressure range, whereby said adhesive may effect rebonding by the mere act of ironing, said adhesive being solid and flexible in use at atmospheric temperatures and remaining substantially solid at 212° F. with resultant ability to avoid migration through the interstices of the fabric layers at the latter temperature, said adhesive being also substantially insoluble in hot water and sufficiently solid to

avoid striking through the fabric under the application of heat and pressure to effect bonding.

14. An article of launderable apparel comprising a plurality of fabric plies united by a pre-formed sheet of thermoplastic synthetic resin which is solid at room temperatures and flexible in thin sheets, said resin being adhesive to said fabric upon becoming softened under the sole action of heat and pressure at normal ironing temperatures and under ironing pressures, and also remaining thermoplastic under repeated heating at ironing temperatures, said resin being also substantially insoluble in hot water and sufficiently flow-resistant at the temperature of boil-

ing water to prevent migration of said substance through the interstices of said fabric.

15. A multi-ply fabric comprising sheets of textile material covering an inner fabric sheet which has been coated on opposite sides with a resin composition consisting essentially of a copolymer of vinyl chloride and vinyl acetate containing a plasticizer which is thermoplastic and resistant to the action of detergents employed in laundering processes, the separate laminae being permanently bonded together by the resin coating of the inner ply into a composite product.

THOMAS H. SWAN.